

## UNITED STATES PATENT OFFICE

2,552,466

## STABILIZED AROMATIC AMINE-GASOLINE MIXTURES

William J. Sweeney, Summit, N. J., assignor to Standard Oil Development Company, a corporation of Delaware

No Drawing. Application March 25, 1948,  
Serial No. 17,110

5 Claims. (Cl. 44—74)

**1** This invention relates to the stabilization of aromatic amines against deterioration by discoloration, etc., during storage. It is particularly directed to the stabilization of aromatic amine-hydrocarbon mixtures, such as gasoline, and is a continuation-in-part of Serial No. 508,394, filed October 30, 1943, now abandoned.

Aromatic amines such as aniline, toluidine, xylidine, etc., are normally substantially colorless when freshly prepared or freshly distilled, but tend to darken in color during storage, the undesirable results being greatly accelerated by storage at elevated temperatures.

The object of the present invention is to stabilize such aromatic amines against discoloration and to stabilize their gasoline fuel blends against gum deposition during storage.

Broadly, the invention comprises adding to the aromatic amines a small amount of a stabilizer comprising an alkyl phenol containing not more than two alkyl groups, at least one of which is in the ortho position (in respect to the hydroxyl group), alone or together with a sulfur-containing stabilizer.

The phenol to be used should usually contain less than about 22, and preferably less than 10, carbon atoms in any one alkyl group, and a total of less than 25, preferably less than 12, alkyl carbon atoms in any one molecule. Dialkyl phenols are preferred. Some specific examples are: 2-tertiary butyl p-cresol, mixed tertiary butyl cresols, 2-methyl p-cresols and other xylenols as well as commercial xlenol products containing large amounts of isomers alkylated in the o-position, petroleum phenols (which are mostly mono- and di-alkylated phenols ranging from 2.6 alkyl C's and averaging about 4 alkyl C's per molecule, with a small amount of alkyl ether derivatives of such phenols, a large amount of such phenols being alkylated in at least one ortho position), o-cresol, 2-isopropyl p-cresol, 2-tertiary amyl p-cresol, 2-secondary amyl p-cresol, o-wax phenol, 2-tertiary butyl 3-methyl phenol, 2-isopropyl 6-methyl phenol, o-isopropyl phenol, o-tertiary butyl phenol, 2-tertiary butyl 4-ethyl phenol, etc. Polynuclear phenols may also be used.

As the optional auxiliary stabilizer, various types of sulfur-containing materials may be used. One class comprises organic sulfur compounds, preferably of the aryl mercaptan type. Such compounds may, for instance, have the general formula

RXH

in which R is an aromatic, preferably an alkyl

aromatic hydrocarbon radical, and X is an atom selected from the group consisting of sulfur, selenium, and tellurium. Although in such compounds it is preferable that R be a mononuclear aromatic radical, i. e., one derived from benzene, poly-nuclear compounds may also be used such as those derived from naphthalene and the like. As mentioned above, it is preferable that the aromatic group R contain one or more

10 alkyl substituents attached to the aromatic nucleus, and in general it is preferable that the radical R contain from 1 to 25 alkyl carbon atoms, preferably 1 to 5 alkyl carbon atoms. One particular sulfur-containing stabilizer which has been

15 found particularly satisfactory is parathiocresol which has the formula  $\text{CH}_3\text{C}_6\text{H}_4\text{SH}$ . Other compounds which may be used include ethylthiophenol, propylthiophenol, various butylthiophenois, such as the paratertiary butylthiophenol,

20 2,4-dimethyl 6-tertiary butyl thiophenol, etc., as well as higher alkyl phenols, e. g., wax thiophenols (in which an alkyl group corresponding to the wax hydrocarbon molecule is attached to the thiophenol nucleus). Other sulfur materials include thiophene and alkylated derivatives thereof, sulfurized mineral oils, carbon disulfide, xanthates, elemental sulfur, etc.

25 Although the amount of the main and optional auxiliary stabilizers to be used may vary according to the intended duration of storage and the temperature of storage, as well as according to the particular aromatic amine and the particular stabilizers used, in general about 0.01% to 1.0% of either stabilizer will be sufficient, and usually about 0.05% to 0.5% by weight of stabilizer will be found most practical for giving satisfactory results.

30 Although the invention is intended to apply broadly to the stabilization of any type of aromatic amines, it is believed particularly applicable to alkaryl amines, especially those having from 1 to 3 alkyl carbon atoms. The invention has been found very successful for the stabilization of xylidine, either the pure separate isomers, or mixtures thereof. Other alkaryl amines which

35 may be stabilized include the toluidines, ortho, meta, or para, or mixtures thereof, the several ethyl anilines, cumidine (which is isopropyl aniline), etc. Dialkylated and trialkylated aryl

40 amines are preferred. Although the invention is particularly applicable to such alkaryl amines, it may also be used for stabilizing aniline, naphthylamines, and the various derivatives of aniline in which either or both of the hydrogens 45 of the amino group are substituted by hydro-

carbons, i. e., either alkyl or aryl groups, e. g., in N-monomethyl aniline, N-dimethyl aniline, N-monoethyl aniline, etc. Thus although the invention is particularly applicable to alkaryl primary amines, other amines such as secondary and tertiary amines may also be used.

The various above described aromatic amines may be used alone as for manufacturing dyes or together with a diluent, such as a hydrocarbon solvent, e. g., naphtha, gasoline for use in motor fuels, aviation fuels, etc. Such diluents may be present in amounts ranging from only a few per cent up to 10, 20 or even 100 times the volume of the aromatic amine.

In carrying out the invention, it is preferred to add the stabilizer(s) to the aromatic amine as soon as the latter has been prepared, or immediately after distillation.

The following experimental data will illustrate the advantages of the invention:

A grade 100/130 aviation gasoline containing 1.0% of two different samples of xylidine, 4-6 ml. of lead tetraethyl and 0.8 lb. /5000 gal. of mixed tertiary butyl para cresol, including 2-tertiary, butyl-4-methyl phenol was subjected to various gum tests and the N<sub>2</sub> bomb test with the following results:

| Xylidine Sample | Inhibitor | Gum Content, Mg./100 ml. |             |            |             | N <sub>2</sub> Bomb Test |
|-----------------|-----------|--------------------------|-------------|------------|-------------|--------------------------|
|                 |           | Glass dish               | Copper dish | 5-Hr. Army | 16-Hr. Army |                          |
| A-----          | No-----   | 3                        | 4           | 7          | 13          | Does not pass.           |
| A-----          | Yes-----  | 2                        | 2           | 6          | 7           | Pass.                    |
| B-----          | No-----   | 2                        | 5           | 7          | 17          | Does not pass.           |
| B-----          | Yes-----  | 1                        | 1           | 5          | 13          | Pass.                    |

It is not intended that this invention be limited to the particular material which have been given merely for the sake of illustration, but only by the appended claims in which it is intended to claim all novelty inherent in the invention as well as all modifications coming within the scope and spirit of the invention.

What is claimed is:

1. A composition comprising gasoline contain-

ing a mononuclear aromatic amine having from 1 to 3 alkyl carbon atoms and a stabilizing amount of a 2,4-dialkyl phenol in which one alkyl substituent is a radical of the group consisting of primary, secondary and tertiary alkyl radicals and the other alkyl substituent is a radical of the group consisting of primary and secondary alkyl radicals.

2. A composition comprising gasoline containing 10 a mononuclear aromatic amine having from 1 to 3 alkyl carbon atoms and a stabilizing amount of a 2,4-dialkyl phenol having a maximum of about 25 carbon atoms and in which one alkyl substituent is a radical of the group consisting of primary, secondary and tertiary alkyl radicals and the other alkyl substituent is a radical of the group consisting of primary and secondary alkyl radicals.

3. A composition comprising gasoline containing 20 at least 1% of a mononuclear aromatic amine having from 1 to 3 alkyl carbon atoms and about 0.0001 to 0.01% by volume of 2,4-dialkyl phenol in which one alkyl substituent is a radical of the group consisting of primary, secondary and tertiary alkyl radicals and the other alkyl substituent is a radical of the group consisting of primary and secondary alkyl radicals.

4. A composition comprising gasoline containing 30 at least 1% of xylidine and about 0.0001 to 0.01% by weight of 2-tertiary butyl paracresol.

5. A composition comprising gasoline containing 35 xylidine and a small amount of mixed mono-tertiary butyl cresols having one of two alkyl groups in the ortho position with respect to a hydroxyl group to stabilize the composition.

WILLIAM J. SWEENEY.

#### REFERENCES CITED

The following references are of record in the 40 file of this patent:

#### UNITED STATES PATENTS

| Number       | Name          | Date          |
|--------------|---------------|---------------|
| 2,410,829    | Luten -----   | Nov. 12, 1946 |
| 45 2,411,307 | Walters ----- | Nov. 19, 1946 |